

1

2,753,265

## PHOTOGRAPHIC DEVELOPING COMPOSITIONS

John David Kendall and Anthony Joseph Axford, Ilford, England, assignors to Ilford Limited, Ilford, England, a British company

No Drawing. Application August 15, 1955,  
Serial No. 528,547

Claims priority, application Great Britain August 24, 1954

15 Claims. (Cl. 95—88)

This invention relates to photographic development and more particularly to photographic developing compositions for the development of images in silver halide photographic emulsions.

In U. S. Patent No. 2,289,367 there is described a new class of photographic developer in which the developing agent, or one of the developing agents, is a 3-pyrazolidone of the formula:



where R<sub>1</sub>, R<sub>2</sub> and R<sub>3</sub> are the same or different and are hydrogen atoms or hydrocarbon groups, for instance alkyl groups, e. g. methyl, ethyl, propyl, isopropyl, or higher alkyl groups, aryl groups, e. g. phenyl or naphthyl groups, or aralkyl groups, e. g. benzyl groups. Such hydrocarbon substituent groups may themselves be substituted; for example, aryl groups may contain hydroxy, alkoxy, aryloxy, oxyalkyl, amino, substituted amino, sulphonic, carboxylic or halogen substituents.

Further, corresponding compounds in which the hydrogen atom in the 4-position of the foregoing formula is substituted by a hydrocarbon group, e. g. the 4,4-dialkyl compounds, have comparable developing activity.

The said specification proposes, inter alia, the formulation of developers containing hydroquinone or pyrogallic acid, which are themselves effective developing agents, in addition to the 3-pyrazolidone.

It has now been discovered that while photographic "glycine," i. e. p-hydroxyphenyl amino acetic acid, has in itself only very weak or negligible developing properties at pH 9 to 10 (which is typical of fine grain developers), except on prolonged development time, and the 3-pyrazolidones alone have but weak developing properties at the same pH values, the two may be employed together to give developing compositions of excellent quality and having important advantages.

According to the present invention, therefore, a developing composition comprises, in alkaline solution (and preferably weakly alkaline solution), p-hydroxyphenyl amino acetic acid and a 3-pyrazolidone. The remarkable results obtained are ascribed to the effect of the 3-pyrazolidone in activating the p-hydroxyphenyl amino acetic acid.

While the broad class of 3-pyrazolidones referred to above are generally useful, the preferred 3-pyrazolidones are the 1-aryl-3-pyrazolidones, and particularly the 1-phenyl-3-pyrazolidones, which are unsubstituted or substituted only by alkyl groups in the 4- and 5-positions. Specific 3-pyrazolidones of value are:

2

1-phenyl-3-pyrazolidone  
1-phenyl-4-methyl-3-pyrazolidone  
1-phenyl-4-ethyl-3-pyrazolidone  
1-phenyl-5-methyl-3-pyrazolidone  
5 1-phenyl-4,4-dimethyl-3-pyrazolidone

The developing compositions according to this invention afford fine grain images of relatively soft gradation and excellent photographic quality. They may be formulated as highly concentrated solutions adapted to be considerably diluted by the user to obtain solutions of working strength.

The following examples will serve to illustrate the invention:

### EXAMPLE 1

#### Developer composition

|                                   | G.  |
|-----------------------------------|-----|
| p-Hydroxyphenyl amino acetic acid | 5   |
| 1-phenyl-3-pyrazolidone           | 0.2 |
| Sodium sulphite (anhydrous)       | 90  |
| Borax                             | 2   |
| Sodium carbonate (anhydrous)      | 2   |
| Water to make 1 litre.            |     |

25 This solution has a pH of 9.0.

Used in the strength indicated, in the development of a fast panchromatic film, at 68° F. for 12 minutes, it yields an image of gamma about 0.6 and of very fine grain. It has a high photographic speed.

30 A corresponding solution without the 1-phenyl-3-pyrazolidone gave no perceptible image on the film even when development was effected at 78° F. and prolonged for 20 minutes. A corresponding solution without the p-hydroxyphenyl amino acetic acid used at 68° F. for 12 minutes afforded only a very weak image.

### EXAMPLE 2

The developer composition of Example 1 was modified by using, instead of 1-phenyl-3-pyrazolidone, 0.2 g. of 1-phenyl-4-methyl-3-pyrazolidone or 0.3 g. of 1-phenyl-4,4-dimethyl-3-pyrazolidone, and each gave very similar results.

### EXAMPLE 3

#### Concentrated developer

|                                     |     |     |
|-------------------------------------|-----|-----|
| Potassium sulphite solution 71% w/v | ml. | 422 |
| p-Hydroxyphenyl amino acetic acid   | g.  | 40  |
| 1-phenyl-3-pyrazolidone             | g.  | 2   |
| 50 Water to make 1 litre.           |     |     |

To this solution was added solid caustic soda in quantity sufficient (usually about 13 g.) to bring the solution, after dilution with 9 parts of water, to a pH of 9.1.

55 In use, this developer is diluted with 9 volumes of water and applied to exposed photographic fast panchromatic film for 10 minutes at 68° F. A fine grain image of gamma about 0.6 is obtained. The developer has a high photographic speed. If the 1-phenyl-3-pyrazolidone is omitted a negligible image is obtained even after 30 minutes at 68° F.

60 It may be observed that a comparable concentrated solution using metol (p-methylamino phenol sulphate) instead of the 3-pyrazolidone cannot be formulated because, to achieve similar photographic results, 15-20 g. of p-methylamino phenol sulphate are required and such a quantity would not remain in the concentrated solution.

65 The foregoing developer, when diluted as indicated, can be kept in full stoppered bottles for three or more months without any substantial loss of developing activity.

## 3

## EXAMPLE 4

|                                         |    |      |
|-----------------------------------------|----|------|
| Potassium sulphite solution 74.3% w./v. | ml | 400  |
| p-Hydroxyphenyl amino acetic acid       | g  | 50   |
| 1-phenyl-3-pyrazolidone                 | g  | 1.75 |
| Potassium bromide                       | g  | 8    |
| Water to make 1 litre.                  |    |      |

Sufficient potassium hydroxide is added so that the pH of the developer after dilution with 7 parts of water to produce a solution of working strength is 9.9. About 10 34 g. is sufficient.

Used for the development of a panchromatic emulsion this formula produces a gamma of approximately 0.7 in about 7 minutes. It is a clean working developer, giving excellent gradation and fine grain.

It will be understood that the developer compositions of this invention may contain any of the restrainers, stabilizers and alkalies known per set for inclusion in developing compositions, e. g. sodium and potassium carbonates or hydroxides, alkali metal, ammonium and alkylolamine sulphites, sodium and potassium metabisulphites, alkali metal bromides, benzotriazole, mercapto triazole and borax.

What we claim is:

1. A photographic developing composition which comprises an alkaline solution containing p-hydroxyphenyl amino acetic acid and a 3-pyrazolidone.

2. A photographic developing composition which comprises an alkaline solution at pH 9 to 10 containing p-hydroxyphenyl amino acetic acid and a 3-pyrazolidone.

3. A photographic developing composition which comprises an alkaline solution containing p-hydroxyphenyl amino acetic acid and 1-phenyl-3-pyrazolidone.

4. A photographic developing composition which comprises an alkaline solution at pH 9 to 10 containing p-hydroxyphenyl amino acetic acid and 1-phenyl-3-pyrazolidone.

5. A photographic developing composition which comprises an alkaline solution containing p-hydroxyphenyl amino acetic acid and a 3-pyrazolidone, said solution further containing an alkali metal carbonate.

6. A photographic developing composition which comprises an alkaline solution at pH 9 to 10 containing p-hydroxyphenyl amino acetic acid and 1-phenyl-3-pyrazolidone, said solution further containing an alkali metal carbonate.

7. A photographic developing composition which com-

## 4

prises an alkaline solution containing p-hydroxyphenyl amino acetic acid and a 3-pyrazolidone, said solution further containing an alkali sulphite.

8. A photographic developing composition which comprises an alkaline solution at pH 9 to 10 containing p-hydroxyphenyl amino acetic acid and 1-phenyl-3-pyrazolidone, said solution further containing an alkali sulphite.

9. A photographic developing composition which comprises an alkaline solution containing p-hydroxyphenyl amino acetic acid and a 3-pyrazolidone, said solution containing alkali metabisulphite.

10. A photographic developing composition which comprises an alkaline solution at pH 9 to 10 containing p-hydroxyphenyl amino acetic acid and 1-phenyl-3-pyrazolidone, said solution containing alkali metabisulphite.

11. A photographic developing composition which comprises an alkaline solution containing p-hydroxyphenyl amino acetic acid and a 3-pyrazolidone, said solution containing an alkali metal bromide.

12. A photographic developing composition which comprises an alkaline solution at pH 9 to 10 containing p-hydroxyphenyl amino acetic acid and 1-phenyl-3-pyrazolidone, said solution containing an alkali metal bromide.

13. A photographic developing composition which comprises an alkaline solution at pH 9 to 10 containing p-hydroxyphenyl amino acetic acid, 1-phenyl-3-pyrazolidone, alkali sulphite and alkali carbonate.

14. A photographic developing composition which comprises an alkaline solution at pH 9 to 10 containing p-hydroxyphenyl amino acetic acid, 1-phenyl-3-pyrazolidone, alkali sulphite, alkali hydroxide and potassium bromide.

15. A photographic developing composition which comprises the following ingredients substantially in the quantities stated:

|                                   | G.   |
|-----------------------------------|------|
| Potassium sulphite                | 297  |
| p-Hydroxyphenyl amino acetic acid | 50   |
| 1-phenyl-3-pyrazolidone           | 1.75 |
| Potassium bromide                 | 8    |
| Water to make 1 litre.            |      |

together with sufficient potassium hydroxide to bring the pH of the said composition, when 1 part thereof is diluted with 7 parts of water, to pH 9.9.

No references cited.